

# UNITED STATES PATENT OFFICE.

HENRI LIVINGSTON BATES, OF SPRINGFIELD, MASSACHUSETTS.

## AIR-TIGHT-SURFACE-FORMING COMPOUND.

1,129,268.

Specification of Letters Patent. Patented Feb. 23, 1915.

No Drawing.

Application filed March 17, 1913. Serial No. 754,929.

To all whom it may concern:

Be it known that I, HENRI L. BATES, a citizen of the United States, residing at Springfield, in the county of Hampden and State of Massachusetts, have invented a new and useful Air-Tight-Surface-Forming Compound; and I do hereby declare the following to be a full, clear, and exact description of the invention, such as will enable others skilled in the art to which it appertains to make and use the same.

This invention relates to water-proofing compounds.

The object of the invention is to provide a compound for treating textile fabrics whereby to render the same thoroughly water and air proof, without in the least detracting from the flexibility of the treated article, or in any way causing deterioration thereof.

The compound is intended primarily for the treatment of fabrics to adapt them for use in preserving ice; but may be employed for any other surface where found of advantage.

The compound consists of the following ingredients in substantially the proportions specified:

|    |                |              |
|----|----------------|--------------|
| 30 | Paraffin       | One pound    |
|    | Spermaceti     | Two ounces   |
|    | Vaseline       | Three ounces |
|    | Cottonseed oil | Three ounces |
|    | Powdered alum  | Two ounces   |
| 35 | Powdered rosin | Two ounces   |
|    | Baking soda    | One ounce.   |

These materials are placed in a suitable vessel and heated until all are melted and thoroughly mixed.

40 In use the fabric is dipped into the compound while warm, then run through a

clothes wringer to remove the surplus and then dried. In treating the fabric it should be observed that all of the interstices are filled, thus to insure an effective and thoroughly water proof article, and one that will be found of the highest efficiency in preserving ice.

Applicant is aware that air tight surface forming compounds have been used heretofore, therefore the compound herein set forth is not claimed broadly, but it has been found that by uniting the particular ingredients as specified in the formula performs a more efficient and desirable result, particularly in that the paraffin, the soda, alum and the rosin, which together with the vaseline and cotton seed oil thoroughly fills or stops up the pores or openings in the fabric and forms a flexible, yet air tight covering or sheath, and one which will more efficiently preserve ice and the like.

What is claimed is:—

A water proofing compound consisting of paraffin, one pound, spermaceti, two ounces, vaseline, three ounces, cottonseed oil, three ounces, powdered alum, two ounces, powdered rosin, two ounces and baking soda, one ounce, said paraffin, alum, rosin and soda together with the vaseline and cotton seed oil constituting a flexible filling for the openings in a piece of fabric, and also acting as a covering for the fabric to render the same air-proof.

In testimony whereof I have signed my name to this specification in the presence of two subscribing witnesses.

HENRI LIVINGSTON BATES.

Witnesses:

ARTHUR A. BETH,  
SAMUEL A. READ.